

3,203,752

**AFTERTREATMENT OF DYED POLYPROPYLENE FIBERS CONTAINING A METAL COMPOUND WITH METAL COMPLEXES**

Walter Percival Mills, Manchester, William Alexander O'Neill, Harrogate, and Raymond Price, Manchester, England, assignors to Imperial Chemical Industries Limited, London, England, a corporation of Great Britain

No Drawing. Filed Dec. 17, 1962, Ser. No. 244,923  
Claims priority, application Great Britain, Dec. 22, 1961,  
46,033

5 Claims. (Cl. 8—75)

This invention relates to the aftertreatment of dyed fibres and more particularly to a process for aftertreating dyed polyolefine and polyacetal fibres containing metal compounds, in order to improve the fastness of the dyestuff to light.

It is known that polyolefine and polyacetal fibres containing metal compounds may be dyed with metallisable dyestuffs, and that by this means the dyestuff becomes firmly anchored within the fibre.

A process is known for the production of coloured shaped articles of poly- $\alpha$ -olefines, in particular coloured fibres of stereoregular polypropylene, wherein there is incorporated a basic or anionic exchange substance which contains a metal, characterized in that the article is dyed with an acid dyestuff which forms a chelate compound.

A process is also known for the production of coloured shaped articles containing or consisting of polyacetals, wherein there is incorporated a basic or anionic exchange substance which contains a metal, characterised in that the article is dyed with an acid dyestuff which forms a chelate compound.

Among the metals which may be contained in the anionic exchange substances particular mention may be made of zinc, magnesium and calcium since these metals do not discolour or adversely affect the properties of the fibre. Other metals may, however, be contained in the anionic exchange substance.

We have now found that the light fastness of metallisable dyes on polyolefine and polyacetal fibres containing certain metals may be improved by aftertreatment of the dyed fibre with certain chelate compounds of other metals.

According to the invention therefore, we provide a process for improving dyeings of metallisable dyes on polyolefine and polyacetal fibres containing zinc, calcium, magnesium or aluminium compounds which comprises treating said dyeings with a chromium, cobalt, nickel or copper complex of a chelating agent which yields a zinc complex having a stability constant not greater than 12.0.

The term "stability constant" has the meaning attributed to it in "Chemistry of the Metal Chelate Compounds," by Martell and Calvin, published in New York in 1952 by Prentice-Hall, Inc. Methods for the determination of stability constants are described in Chapter 3.

We mention the following chelating agents which yield zinc complexes having stability constants not greater than 12.0. 8-hydroxyquinoline (10.9), acetylacetone (5.6), benzoylacetone (5.6), glycine (5.5), salicylic acid, salicyl-aldehyde (4.5), salicylaldoxime, o-hydroxyacetophenone oxime, ethylene diamine (5.9) and o-phenanthroline (6.4). The chromium, cobalt, nickel and copper complexes of such chelating agents are of value in the process of the invention.

During the process of the invention metal exchange is believed to occur, resulting in the formation of a dyestuff complex of chromium, cobalt, nickel or copper within the polypropylene fibre. It is surprising that metal exchange can be brought about so readily in a completely non-polar medium such as polypropylene. The remark-

able increases in light fastness which we are able to produce are in themselves evidence that a considerable amount of metal exchange takes place.

The chromium, cobalt, nickel and copper complexes of acetylacetone are especially valuable in the process of the invention, being stable under ordinary conditions of storage and in aqueous dispersion, but sufficiently reactive with the dyed fibre to produce rapid and extensive metal exchange under the conditions described above.

10 The process of our invention may conveniently be carried out by treatment of the dyeing with an aqueous dispersion of the chromium, cobalt, nickel or copper complex (obtained, for example, by milling the complex with an aqueous solution of a dispersing agent such as a sulphonated naphthalene-formaldehyde condensate). Such treatment may readily be carried out at a temperature between 70° C. and 120° C., especially between 80° and 100° C. The process is usually complete after heating for about 1 hour between 80° and 100° C., and the textile material may then be rinsed, treated with soap or detergent in normal manner and dried.

15 Dyed polyolefine or polyacetal fibres suitable for aftertreatment with metal complexes by the process of the invention may be obtained according to known processes generally described above. It is especially advantageous to use a sequestering agent at some stage of the dyeing operation. Particularly, dyed fibres of stereoregular polypropylene containing the said metal compounds may be used in the process of our invention. The zinc, calcium, magnesium or aluminium compounds contained in such fibres are preferably salts of high molecular weight carboxylic acids e.g. 8 to 18 carbon atoms carboxylic acids such as caprylic, stearic or naphthenic acids. Other metal compounds such as inorganic salts and oxides may be contained in the fibres if desired.

20 The invention is of great value when it is applied to dyeings of metallisable dyestuffs on polyolefine and polyacetal fibres containing compounds of zinc, magnesium or calcium. Such dyeings, especially when obtained from metallisable dyestuffs of the monoazo or anthraquinone series are normally of low fastness to light, and aftertreatment with the metal chelate compound brings about a marked improvement. A very marked improvement in light fastness occurs when the dyestuff used is a monoazo dyestuff containing metal-reactive (especially hydroxy) groups in positions ortho- to the azo group.

25 The invention is illustrated but not limited by the following examples in which the parts are by weights. The light fastness figures are those obtained by the method adopted by the International Organization for Standardization (I.S.O. Recommendation R 105, Part II). The method of testing is also described in "British Standards," under BS 1006.

*Example 1*

30 55 100 parts of a polypropylene textile material containing 95% isotactic polypropylene and 5% zinc stearate is scoured for 30 minutes at 85° C. in a bath containing 0.2 part of sodium oleyl p-anisidine sulphonate and 2 parts of ethylene diamine tetraacetic acid sodium salt per 1000 parts water, and rinsed thoroughly in water.

35 60 1.5 parts of 1-(2'-hydroxyphenylazo)-2-naphthol is dispersed in water by gravel milling with 0.3 part of a sulphonated naphthalene - formaldehyde condensation product, and added to 4000 parts of water at 50° C. containing 4 parts sulphonated naphthalene-formaldehyde condensation product. The scoured polypropylene textile material is immersed in the liquid thus obtained and the temperature is raised to 100° C. Dyeing is continued for 90 minutes at 100° C. and the textile material is then rinsed in water. The deep red textile material is then after-treated by immersion in 4000 parts of warm water con-

taining 2 parts of the copper complex of 8-hydroxyquinoline (dispersed by gravel milling with 0.5 parts of sulphonated naphthalene-formaldehyde condensation product and 10 parts of water) and 4 parts of sulphonated naphthalene formaldehyde condensation product. The temperature is raised to 85° C. for 1 hour and the textile material is rinsed in water and washed for 15 minutes at 60° C. in a solution of a synthetic detergent and finally rinsed in water and dried.

The dyeing so obtained has a light fastness of 5. If the aftertreatment with the copper complex is omitted, the dyeing has a light fastness of 2.

*Example 2*

Example 1 is repeated using a polypropylene textile material containing 95% isotactic polypropylene and 5% magnesium naphthenate. The dyeing so obtained has a light fastness between 4 and 5. If the aftertreatment with

the copper complex is omitted the dyeing has a light fastness between 1 and 2.

*Example 3*

Example 1 is repeated using a polypropylene textile material containing 95% isotactic polypropylene and 5% calcium oxide. The dyeing so obtained has a light fastness of 4. If the aftertreatment with the copper complex is omitted the dyeing has a light fastness of 1.

The following tables give further examples, indicating in column 5 the shades obtained on polypropylene textile material containing 95% isotactic polypropylene and 5% zinc stearate by dyeing with the dyestuffs listed in column 2 and aftertreating with an aqueous dispersion of the metal complexes listed in column 4, using the procedures described in Example 1. The light fastness figures, before and after the treatment with the metal complex are given in columns 3 and 6 respectively.

TABLE I

| Example | Dyestuff                                     | Light fastness | Metal complex                      | Shade      | Light fastness after treatment |
|---------|----------------------------------------------|----------------|------------------------------------|------------|--------------------------------|
| 4       | 1-(quinoline-8'-azo)-2-naphthol              | 2-3            | Copper/8-hydroxyquinoline          | Rubine     | 4                              |
| 5       | 1-(2'-hydroxyphenylazo)-2-naphthol           | 2              | Copper/acetyl acetone              | Deep red   | 5                              |
| 6       | do                                           | 2              | Copper/salicylic acid              | do         | 4-5                            |
| 7       | do                                           | 2              | Cobalt/acetyl acetone              | do         | 5                              |
| 8       | do                                           | 2              | Chromium/8-hydroxyquinoline        | do         | 4                              |
| 9       | 1-(2'-hydroxy-3'-chlorophenylazo)-2-naphthol | 3              | Copper/8-hydroxyquinoline          | Bluish red | 6                              |
| 10      | do                                           | 3              | Copper/salicylaldoxime             | do         | 6                              |
| 11      | 1-(2'-hydroxy-5'-chlorophenylazo)-2-naphthol | 4              | Copper/8-hydroxyquinoline          | do         | 5-6                            |
| 12      | do                                           | 4              | Copper/o-hydroxyacetophenone oxime | do         | 5-6                            |

TABLE II

| Example | Metal compound        | Dyestuff                                                                | Light fastness | Metal complex                        | Shade      | Light fastness after treatment |
|---------|-----------------------|-------------------------------------------------------------------------|----------------|--------------------------------------|------------|--------------------------------|
| 13      | Zinc stearate         | 2':4'-Dichloro-2-hydroxy-5-methylazobenzene                             | 4              | Copper/acetyl acetone                | Yellow     | 5                              |
| 14      | do                    | 1-(4'-Methoxyphenylazo)-2-naphthol                                      | 2-3            | do                                   | Pink       | 4                              |
| 15      | do                    | 1-(2'-Carboxyphenylazo)-2-naphthol                                      | 2-3            | Copper/salicylaldoxime               | Red        | 4                              |
| 16      | do                    | 1-(2'-Methoxyphenylazo)-2-naphthol                                      | 2-3            | Copper/o-hydroxyacetophenone oxime   | Pink       | 4                              |
| 17      | Calcium stearate      | 1-(2'-hydroxy-5'-chlorophenylazo)-2-naphthol                            | 4              | Chromium/acetyl acetone              | Bluish red | 5                              |
| 18      | Zinc naphthenate      | 1-(2'-Hydroxy-5'-chlorophenylazo)-2-naphthol                            | 4              | Copper/ethylene diamine              | do         | 5-6                            |
| 19      | Zinc stearate         | 1-Phenyl-3-ethoxycarbonyl-4-(2'-hydroxyphenylazo)-5-pyrazolone          | 3-4            | Copper/glycine                       | Yellow     | 4                              |
| 20      | do                    | 1-Phenyl-3-ethoxycarbonyl-4-(4'-nitro-2'-hydroxyphenylazo)-5-pyrazolone | 2              | Copper/benzoyl acetone               | Orange     | 4                              |
| 21      | do                    | 1-(4'-chlorophenyl)-3-methyl-4-(2'-hydroxyphenylazo)-5-pyrazolone       | 2              | Copper/acetyl acetone                | Yellow     | 4                              |
| 22      | Zinc naphthenate      | 1-Phenyl-3-ethoxycarbonyl-4-(2'-hydroxyphenylazo)-5-pyrazolone          | 3-4            | Copper/3-dodecylpentane-2:4-dione    | do         | 4-5                            |
| 23      | do                    | 1-Phenyl-3-ethoxycarbonyl-4-(2'-hydroxyphenylazo)-5-pyrazolone          | 3-4            | Copper/5-dodecyl-5-hydroxyquinoline  | do         | 4-5                            |
| 24      | do                    | do                                                                      | 3-4            | Copper/5-n-propyl-8-hydroxyquinoline | do         | 4-5                            |
| 25      | Magnesium naphthenate | 5-(4'-Diethylaminophenylazo)-8-hydroxyquinoline                         | 2              | Copper/methylacetone                 | Red        | 4                              |
| 26      | Zinc octoate          | 5-(2'-ethoxy-4'-diethylaminophenylazo)-8-hydroxyquinoline               | 3              | Cobalt/3-n-butylpentane 2:4-dione    | do         | 5                              |
| 27      | do                    | 5-(4'-chloro-2'-methylphenylazo)-8-hydroxyquinoline                     | 4              | Copper/o-phenanthroline              | Orange     | 5-6                            |
| 28      | Magnesium naphthenate | 5-(2':4'-dichlorophenylazo)-8-hydroxyquinoline                          | 4              | Cobalt/benzoylacetone                | do         | 5-6                            |
| 29      | do                    | 5-(4'-methylphenylazo)-8-hydroxyquinoline                               | 4              | Nickel/acetylacetone                 | do         | 5-6                            |
| 30      | Zinc stearate         | 1-(4'-diethylaminophenylazo)-4-hydroxyacridine                          | 2              | Copper/acetylacetone                 | Brown      | 4                              |
| 31      | do                    | 1-(4'-phenylbenzeneazo)-4-hydroxyacridine                               | 3              | Nickel/acetylacetone                 | do         | 4-5                            |
| 32      | do                    | 7(4'-n-butylphenylazo)-2-acetylaminoo-4-hydroxybenzthiazole             | 2-3            | do                                   | Yellow     | 5                              |
| 33      | do                    | 7(4'-chlorophenylazo)-2-acetylaminoo-4-hydroxybenzthiazole              | 3              | Copper/8-hydroxyquinoline            | do         | 5                              |
| 34      | do                    | 7(2':4'-dichlorophenylazo)-2-acetylaminoo-4-hydroxybenzthiazole         | 3-4            | Copper/acetylacetone                 | do         | 5-6                            |
| 35      | do                    | 3-oximinomethyl-4-hydroxy-4'-methylazobenzene                           | 2              | do                                   | do         | 4                              |
| 36      | do                    | 3-carboxy-4-hydroxy-4'-nitroazobenzene                                  | 3-4            | do                                   | do         | 5                              |
| 37      | do                    | 3:4-dihydroxy-4'-ethoxyazobenzene                                       | 5-6            | Copper/8-hydroxyquinoline            | Brown      | 4                              |
| 38      | do                    | 1:2-dihydroxy-3-nitroanthraquinone                                      | 5-6            | do                                   | Red-brown  | 6-7                            |
| 39      | do                    | 1:2-dihydroxyanthraquinone                                              | 6              | do                                   | Maroon     | 6-7                            |
| 40      | do                    | 1:5:8-trihydroxy-2-aminoanthraquinone                                   | 4-5            | do                                   | Bordeaux   | 5-6                            |
| 41      | Magnesium stearate    | 1:2-dihydroxy-3-aminoanthraquinone                                      | 4-5            | do                                   | Brown      | 5-6                            |
| 42      | Zinc stearate         | 5:8-di(4'-methylphenylamino)1:2-dihydroxyanthraquinone                  | 5              | do                                   | Blue       | 6                              |
| 43      | do                    | 3-cyano-1:5-di(o-hydroxyphenyl) formazan                                | 2              | Copper/ethylene diamine              | do         | 4                              |

We claim:

1. A process for improving dyeings of dyestuffs selected from the class consisting of metallisable dyestuffs of the monoazo- and anthraquinone series on stereoregular polypropylene fibres containing metal compounds selected from the class consisting of zinc, calcium, magnesium and aluminum salts of eight to eighteen carbon atom carboxylic acids which comprises immersing said dyeings in an aqueous dispersion of a metal complex selected from the class consisting of chromium, cobalt, nickel and copper complexes of chelating agents, which chelating agents yield zinc complexes having stability constants of at least 4.0 and at most 12.0, at a temperature between 70° and 120° C.

2. A process for improving dyeings of monoazo dyestuffs having hydroxy groups in positions ortho to the azo group on stereoregular polypropylene fibres containing a zinc salt of an 8 to 18 carbon atom carboxylic acid which comprises immersing said dyeings in an aqueous dispersion of a copper complex of a chelating agent, which chelating agent yields a zinc complex having a stability constant of at least 4.0 and at most 12.0, at a temperature between 70° and 120° C.

3. A process for improving dyeings of monoazo dyestuffs having hydroxy groups in positions ortho to the azo group on stereoregular polypropylene fibres containing a zinc salt of an 8 to 18 carbon atom carboxylic acid which comprises immersing said dyeings in an aqueous dispersion of a copper complex of acetylacetone at a temperature between 70° and 120° C.

4. A process for improving dyeing of dyestuffs selected from the class consisting of metallisable dyestuffs of the monoazo- and anthraquinone series on stereoregular polypropylene fibres containing a zinc salt of eight to

eighteen carbon atom carboxylic acids with comprises immersing said dyeings in an aqueous dispersion of a metal complex selected from the class consisting of chromium, cobalt, nickel and copper complexes of chelating agents, which chelating agents yield zinc complexes having stability constants of up to about 12.0 at a temperature within the range of about 70° to about 120° C.

5. A process for improving dyeings of dyestuffs selected from the class consisting of metallisable dyestuffs of the monoazo- and anthraquinone series on stereoregular polypropylene fibres containing metal compounds selected from the class consisting of zinc, calcium, magnesium and aluminum salts of eight to eighteen carbon atom carboxylic acids which comprises immersing said dyeings in an aqueous dispersion of a metal complex selected from the class consisting of chromium, cobalt, nickel and copper complexes of chelating agent, which chelating agents yield zinc complexes having stability constants of at most 12.0, at a temperature between 70° and 120° C.

#### References Cited by the Examiner

##### UNITED STATES PATENTS

|              |       |                 |       |        |
|--------------|-------|-----------------|-------|--------|
| 120,393      | 10/71 | Raraf           | ----- | 8—29   |
| 1,805,467    | 5/31  | Dreyfus         | ----- | 8—31   |
| 25 1,896,381 | 2/33  | Weber et al.    | ----- | 8—95   |
| 1,947,597    | 2/34  | Hoelkeskamp     | ----- | 8—95   |
| 2,215,196    | 9/40  | Schlack         | ----- | 8—29   |
| 2,945,010    | 7/60  | Caldwell et al. | ----- | 8—99 X |
| 2,984,634    | 5/61  | Caldwell et al. | ----- | 8—99   |
| 30 3,008,858 | 11/61 | Blake et al.    | ----- |        |

NORMAN G. TORCHIN, *Primary Examiner.*

ABRAHAM H. WINKELSTEIN, *Examiner.*